

## [54] HEAT-SENSITIVE COPY-SHEET

[75] Inventor: Kevin P. O'Leary, Minneapolis, Minn.

[73] Assignee: Minnesota Mining &amp; Manufacturing Company, St. Paul, Minn.

[22] Filed: Dec. 13, 1972

[21] Appl. No.: 314,687

[52] U.S. Cl. .... 117/36.8, 117/36.9, 260/65 T

[51] Int. Cl. .... B41m 5/00

[58] Field of Search: 117/36.9, 36.2, 36.8; 8/10.2; 250/65 T

## [56] References Cited

## UNITED STATES PATENTS

3,609,360 9/1971 Wiese ..... 250/65 T

|           |         |                                   |
|-----------|---------|-----------------------------------|
| 3,682,684 | 8/1972  | Newman et al. .... 117/36.9       |
| 3,684,552 | 8/1972  | Wiese et al. .... 117/36.8        |
| 3,715,213 | 2/1973  | Nihyakumen et al. .... 117/36.9 X |
| 3,730,677 | 5/1973  | Kalopissis et al. .... 8/10.2     |
| 3,751,249 | 8/1973  | Hiller .... 117/36.8 X            |
| 3,764,333 | 10/1973 | Leclair et al. .... 117/36.9 X    |

Primary Examiner—Thomas J. Herbert, Jr.

Attorney, Agent, or Firm—Alexander, Sell, Steldt &amp; DeLaHunt

## [57] ABSTRACT

A transparent colored film product, which becomes clear and colorless at image areas when heated thermographically, contains a p-quinoneimine color body and a mild reducing agent.

7 Claims, No Drawings

## HEAT-SENSITIVE COPY-SHEET

This invention relates to thermographic copying, wherein a copy of a differentially radiation-absorptive original is made on a heat-sensitive copy-sheet product held in heat-conductive contact therewith by briefly exposing the original to intense infra-red radiation. In one aspect the invention relates to novel heat-sensitive copy-sheet products. In a particularly important aspect the invention relates to copy-sheet products useful in making negative color projection transparencies.

Negative-acting copy-sheets adapted for making color projection transparencies have previously been described. In U.S. Pat. No. 3,609,360 the decolorization involves the heat-induced decomposition of a colored reaction product of components including a volatile acid which is then released to the atmosphere. U.S. Pat. No. 3,684,552 somewhat analogously uses an amine-reactive color body and a heat-decomposable salt of a nitrogenous organic base.

The present invention employs a different class of color bodies and a different reaction system, and provides a heat-sensitive copy-sheet product which when locally heated, as in the thermographic copying process, is converted from a highly colored to a substantially colorless, and preferably a clear and transparent, form at the heated image areas without release of volatile decomposition products.

The heat-sensitive copy-sheet products of the present invention contain p-quinoneimine color bodies which undergo decolorization when heated at thermographically induced temperatures in reactive association with a mild reducing agent. The color body is supplied in a matrix of film-forming binder as a coating on a paper, transparent film or other carrier or as a self-supporting film. The reducing agent may be incorporated in the same matrix, or in an adjacent stratum supported on the carrier or on a separate carrier. A particularly useful structure comprises a transparent flexible film carrier coated with a first stratum of p-quinoneimine color body in a transparent binder and overcoated with a mild reducing agent in a separate binder. Brief heating of the film product causes migration of at least one of the reactants and results in a decolorization of the color body at the heated area.

Reducible p-quinoneimine color bodies which are useful in the preparation of heat-sensitive copy-sheets of the invention include those having the structural formula



wherein Ar is an aromatic radical and the R, R', R'' and R''' substituent radicals may be hydrogen, halogen, alkyl, alkoxy or amido, or wherein substituent radicals on adjacent carbon atoms may complete a fused polycyclic or heterocyclic ring, all as exemplified by the following illustrative compounds:

- 2-methyl-N(p-morpholinophenyl)-p-  
benzquinoneimine  
2,6-dimethyl-N(p-morpholinophenyl)-p-  
benzoquinoneimine  
2,6-dichloro-N(p-morpholinophenyl)-p-  
benzoquinoneimine

- 2-chloro-2'-methyl-N,N-diethylindoaniline  
2-chloro-N(p-diethylamino-2-methylphenyl)-p-  
benzoquinoneimine  
2-acetamido-N,N-diethylindoaniline  
3-methoxy-2'-methyl-N,N-diethylindoaniline  
N-(1-naphthyl)-p-benzoquinoneimine  
N-(2-naphthyl)-p-benzoquinoneimine  
N-(p-acetylphenyl)-p-benzoquinoneimine  
2,6-dichloroindophenol sodium salt  
2,3',6-trichloroindophenol sodium salt  
2,6-dibromoindophenol sodium salt  
2,5-dibromo-N(2,4-dibromophenyl)-p-  
benzoquinoneimine  
N-(p-diethylamino-2-methylphenyl)-1,4-  
naphthoquinoneimine  
N-(p-diethylamino-2-methylphenyl)-5,8-  
quinolinoquinoneimine  
N-(2,4-diamino-5-methylphenyl)-p-  
benzoquinoneimine trihydrate indoferron  
N-(p-diethylamino-2-methylphenyl)-2-carboxylic-1,  
4-naphthoquinoneimine  
N-(p-dimethylaminophenyl)-1,4-  
naphthoquinoneimine  
The following mild reducing agents have been found  
useful:  
2,5-dihydroxybenzoic acid  
chlorohydroquinone  
2,5-dichlorohydroquinone  
30 tetrachlorohydroquinone  
bromohydroquinone  
diiodohydroquinone  
phenylhydroquinone  
2,6-di-t-butylhydroquinone  
2,5-di-t-butylhydroquinone  
35 2,5 bis(1,1-dimethylpropyl) hydroquinone  
2,5-di-pentylhydroquinone  
trimethylhydroquinone  
t-butylhydroquinone  
methylhydroquinone  
catechol  
3-methylcatechol  
4-methylcatechol  
4-t-butylcatechol  
3-isopropylcatechol  
4-isopropylcatechol  
45 4-t-octylcatechol  
3,5-diisopropylcatechol  
3,6-diisopropylcatechol  
3,5-di-t-butylcatechol  
3-t-butyl-5-methylcatechol  
3-methyl-5-t-butylcatechol  
3-methyl-5-octylcatechol  
3-methoxycatechol  
50 tetrabromocatechol  
resorcinol  
4-ethylresorcinol  
4-n-propylresorcinol  
4'-phenylazoresorcinol  
4,6-dichlororesorcinol  
o-hydroxyethylresorcinol  
2,6-dihydroxybenzoic acid  
2,4-dihydroxybenzaldehyde  
2', 6'-dihydroxyacetophenone  
2', 4', 6'-trihydroxyacetophenone  
60 methyl gallate  
butyl gallate  
1,2,3-trihydroxybenzene

2',3',4'-trihydroxydecanophenone  
 1,2,4-trihydroxybenzene  
 2,4,5-trihydroxybutyrophenone  
 o-aminophenol  
 m-aminophenol  
 p-aminophenol  
 4-amino-2,6-dibromophenol  
 4-amino-2,6-dichlorophenol  
 2-amino-4-chlorophenol  
 3-diethylaminophenol  
 2,4-diaminophenol  
 p-benzylaminophenol  
 4-amino-2,5-dimethylphenol  
 6-amino-m-cresol  
 4-amino-m-cresol  
 5-amino-1-naphthol  
 m-hydroxydiphenylamine  
 4'-aminoacetanilide  
 2,6-diaminotoluene  
 3,4-diaminotoluene  
 1,4-diaminobenzene  
 1,8-diaminonaphthalene  
 tetramethyl-1,4-diaminobenzene  
 furoin  
 1,3-dihydroxyacetone  
 L-ascorbic acid  
 arabo-ascorbic acid  
 4-methoxy-1-naphthol  
 2-methoxy-1-naphthol  
 1-amino-2-methoxynaphthalene  
 2,3-naphthalene diol  
 1,4-naphthalene diol  
 5,8-dihydroxy-1,4-dihydro-2-methylnaphthalene  
 1-naphthol

Strong reducing agents may also be used in some cases, in particular with the lower molecular weight color bodies and in constructions involving separate sheets, but are presently of only minor interest.

Binder systems may include such polymeric materials as polystyrene, styrene-acrylonitrile or styrene-acrylate copolymers, styrene-butadiene-acrylonitrile terpolymers, polyvinylchloride, vinyl chloride-vinyl acetate copolymers, vinylidene chloride-acrylonitrile or vinylidene chloride-vinyl acetate copolymers, polyacrylates, polyvinyltoluene. These polymers are moisture-resistant, being incapable of absorbing more than about one percent of water, and are preferred as contributing to the stability of the sheet materials during prolonged storage both before and after imaging.

The concentration of color body in the color stratum must be sufficient to impart a distinctive color but excessive amounts require undesirably large quantities of reducing agent, or excessive heating, or may reduce the transparency of the stratum and accordingly are to be avoided. Similarly, the amount of reducing agent available per unit area should be sufficient to react with all of the color body but need not be greatly in excess of that amount and, at least for single sheet projection transparencies, should be well within the range of full compatibility with the binder so that the stratum remains clear and non-light-diffusing.

The following Examples, in which all proportions are in parts by weight unless otherwise indicated, will further illustrate the practice of the invention which however is not to be construed as limited thereto.

## EXAMPLE 1

A carrier film of 2 mil (0.05 mm.) ethylene glycol terephthalate polyester film primed with a trace coating of terpolymer primer is supplied with first and second reactant strata, with intermediate and final drying, as follows:

|    |                                                                                                                                                                                                                                                                         |      |
|----|-------------------------------------------------------------------------------------------------------------------------------------------------------------------------------------------------------------------------------------------------------------------------|------|
| 10 | First stratum                                                                                                                                                                                                                                                           |      |
|    | 2-chloro-2'-methyl-N,N-diethylindoaniline                                                                                                                                                                                                                               | 1.6  |
|    | polyvinyl chloride-acetate ("Geon 421" resin)                                                                                                                                                                                                                           | 11.8 |
|    | methyl ethyl ketone                                                                                                                                                                                                                                                     | 69.3 |
|    | toluene                                                                                                                                                                                                                                                                 | 17.3 |
|    | dry at 180°F.                                                                                                                                                                                                                                                           |      |
|    | coating weight, dry, 2.5 g./sq. m.                                                                                                                                                                                                                                      |      |
| 15 | Second stratum                                                                                                                                                                                                                                                          |      |
|    | tertiarybutylhydroquinone                                                                                                                                                                                                                                               | 4.4  |
|    | polyvinyl butyral ("Butvar B-76" resin)                                                                                                                                                                                                                                 | 2.6  |
|    | nitrocellulose (½ sec.)                                                                                                                                                                                                                                                 | 10.4 |
|    | methanol                                                                                                                                                                                                                                                                | 82.6 |
|    | dry at 130°F.                                                                                                                                                                                                                                                           |      |
|    | coating weight, dry, 4.0 g./sq. m.                                                                                                                                                                                                                                      |      |
| 20 |                                                                                                                                                                                                                                                                         |      |
|    | The resulting sheet is transparent and blue in color.                                                                                                                                                                                                                   |      |
|    | It is placed against an original consisting of line drawings in black ink or a white paper and the composite is passed through a thermographic copy machine. The                                                                                                        |      |
| 25 | blue color disappears at the heated image areas. The sheet is placed on an overhead projector and is found to project a white image on a blue background. The appearance of the sheet and of the projected pattern remains unchanged during several hours of continuous |      |
| 30 | projection.                                                                                                                                                                                                                                                             |      |

## EXAMPLE 2

A solution containing

|    |                                            |      |
|----|--------------------------------------------|------|
| 35 | 2-chloro-2'-methyl-N,N-dimethylindoaniline | 0.6  |
|    | polyvinyl chloride-acetate ("VYNS" resin)  | 12.0 |
|    | methyl ethyl ketone                        | 96   |
|    | toluene                                    | 12   |

is applied to thin polyester film and dried in an oven at 150°F. The dried coating is a deep blue in color and weighs 4.7 g./sq. m.

A solution containing

|    |                                   |    |
|----|-----------------------------------|----|
| 45 | tertiary butyl hydroquinone       | 1  |
|    | ½ sec. nitrocellulose             | 1  |
|    | polyamide ("Elvamide 8061" resin) | 1  |
|    | methanol                          | 97 |

is applied over the first coating at approximately the same wet coating thickness and is promptly dried in the 150°F. oven.

The resulting film is imaged in a thermographic copying machine to provide a negative color projection transparency as in Example 1.

## EXAMPLE 3

|    |                                               |      |
|----|-----------------------------------------------|------|
| 60 | First trip solution                           |      |
|    | 2-chloro-2'-methyl-N,N-diethylindoaniline     | 0.25 |
|    | polystyrene ("Styron 690" resin)              | 7.5  |
|    | methyl ethyl ketone                           | 42.5 |
|    | Second trip solution                          |      |
|    | tertiarybutyl hydroquinone                    | 0.67 |
|    | 13.5% solution of nitrocellulose in methanol  | 8    |
|    | 13.5% solution of polyvinylbutyral in ethanol | 2    |

Coating weights and procedures are as described in previous Examples. By thermographic copying a good negative color projection transparency is obtained.

## EXAMPLE 4

|                                                   |      |  |  |
|---------------------------------------------------|------|--|--|
| First trip solution                               |      |  |  |
| 2-chloro-2'-methyl-N,N-diethylindoaniline         | 0.50 |  |  |
| vinyl chloride-acetate polymer ("Geon 421" resin) | 7.5  |  |  |
| acetone                                           | 67.5 |  |  |
| Second trip solution                              |      |  |  |
| t-butyl hydroquinone                              | 1.3  |  |  |
| ethyl cellulose ("G-200" resin)                   | 5    |  |  |
| ethanol                                           | 95   |  |  |

Procedures and results are generally as described in preceding Examples.

## EXAMPLE 5

|                                           |      |  |  |
|-------------------------------------------|------|--|--|
| First trip solution                       |      |  |  |
| 2-chloro-2'-methyl-N,N-diethylindoaniline | 0.25 |  |  |
| vinyl chloride-acetate polymer            | 5    |  |  |
| methyl ethyl ketone                       | 36   |  |  |
| toluene                                   | 9    |  |  |
| Second trip solution                      |      |  |  |
| t-butyl hydroquinone                      | 5    |  |  |
| methanol                                  | 35   |  |  |
| acrylate latex ("Rhoplex AC-61"), 45% NVM | 36   |  |  |
| colloidal silica ("Ludox AM")             | 24   |  |  |

Introduction of silica improves the resistance of the coating to surface picking and roughening during thermographic copying without appreciably reducing the clarity. Procedures and results are substantially as described in the preceding Examples.

## EXAMPLE 6

|                                           |      |    |  |
|-------------------------------------------|------|----|--|
| Solution A                                |      |    |  |
| N-(p-acetylphenyl)-p-benzoquinoneimine    | 0.4  |    |  |
| polyvinyl chloride-acetate ("VYNS" resin) | 5    |    |  |
| methyl ethyl ketone                       | 40.5 | 35 |  |
| toluene                                   | 4.5  |    |  |
| Solution B                                |      |    |  |
| methyl hydroquinone                       | 10   |    |  |
| polyvinyl chloride-acetate ("VYHH" resin) | 2    |    |  |
| polyvinyl butyral ("Butvar B-76" resin)   | 10   |    |  |
| methyl ethyl ketone                       | 76   |    |  |

Solution A is applied to thin 2 mil (0.05 mm.) polyester film from a coater bar at a 2 mil (0.05 mm.) orifice and the coating is dried. Similarly, solution B is coated at the same thickness on a separate portion of 1 mil (0.025 mm.) film and the coating is dried. The two sheets are placed in face-to-face contact. The composite is placed against a printed original which is then subjected to brief exposure to intense infra-red radiation. The second sheet is peeled from the first, leaving a projection transparency with clear image areas and yellow background areas.

## EXAMPLE 7

|                                           |      |  |  |
|-------------------------------------------|------|--|--|
| Solution A                                |      |  |  |
| 2-chloro-2'-methyl-N,N-diethylindoaniline | 0.25 |  |  |
| polyvinyl chloride-acetate                | 5    |  |  |
| methyl ethyl ketone                       | 40.5 |  |  |
| toluene                                   | 4.5  |  |  |
| Solution B                                |      |  |  |
| t-butyl hydroquinone                      | 10   |  |  |
| ethyl cellulose ("T-100" resin)           | 10   |  |  |
| ethanol                                   | 80   |  |  |

The solutions are coated on separate sheets of thin polyester film, and the two sheets are combined and processed, as in Example 6, with similar results.

As an alternate structure a second sheet is prepared from a solution of ten parts of t-butyl hydroquinone

and 9 parts of polyvinyl butyral resin in 91 parts of acetone, coated on thin (21 1/2 lb/ream) glassine. Substantially the same results are obtained.

## EXAMPLE 8

## First coat

|                                           |      |
|-------------------------------------------|------|
| 2-chloro-2'-methyl-N,N-diethylindoaniline | 0.25 |
| polyvinyl chloride-acetate                | 10   |
| methyl ethyl ketone                       | 90   |

## 15 Second coat

|                          |     |
|--------------------------|-----|
| 4-methoxy-1-naphthol     | 15  |
| polyvinyl butyral        | 30  |
| titanium dioxide pigment | 10  |
| ethanol                  | 222 |

The mixture is homogenized by prolonged milling in a ball mill, applied over the first coat at the same orifice, and dried.

The coated sheet provides a white image against an opaque blue background when used as a thermographic copy-sheet.

## EXAMPLE 9

## 30 First coat

|                 |    |
|-----------------|----|
| methyl gallate  | 3  |
| ethyl cellulose | 5  |
| ethanol         | 95 |

Coated on 2 mil (0.05 mm.) polyester film at 2 mil (0.05 mm.) orifice, and dried.

## Second coat

|                                               |     |
|-----------------------------------------------|-----|
| 2,6-dichloroindophenol sodium salt            | 0.3 |
| polystyrene-acrylonitrile ("Tyril 860" resin) | 15  |
| acetone                                       | 85  |

Coated over first coat at 2 mils (0.05 mm.) and dried.

The product provides a negative color projection transparency by thermographic copying.

## EXAMPLE 10

55 To a solution of 0.08 part 2,6-dichloro-N(p-morpholinophenyl)-p-benzoquinoneimine and 5 parts of a copolymer of methyl methacrylate and ethyl acrylate in 20 parts of methyl ethyl ketone is added 0.45 part of 2,5-dihydroxybenzoic acid and the mixture is quickly coated on transparent film and dried. The sheet provides a color projection transparency when printed thermographically but is found to have short shelf life, the initial magenta color gradually fading during storage. Some improvement in performance may be achieved by increasing the proportion of binder but these sheets are generally less permanent and hence less desirable than those in which the two reactants are in separate strata.

## EXAMPLE 11

|                                                              |      |
|--------------------------------------------------------------|------|
| First solution                                               |      |
| N-(p-diethylamino-2-methylphenyl)-5,8-quinolino quinoneimine | 0.25 |
| polyvinyl chloride-acetate                                   | 6    |
| methylethyl ketone                                           | 44   |
| nickel resinate                                              | q.v. |
| Second solution                                              |      |
| tertiarybutyl hydroquinone                                   | 0.67 |
| 13.5% solution of nitrocellulose in methanol                 | 8    |
| 13.5% solution of polyvinylbutyral in ethanol                | 2    |

Sufficient nickel resinate solution is added in the first solution to change the color from blue to green. The solution is coated on polyester film at 0.05 mm. and dried, and is overcoated with an equal wet thickness of the second solution which is also promptly dried. Under thermographic copying procedures the sheet provides a color projection transparency with clear image areas and a green background.

## EXAMPLE 12

|                                                |      |
|------------------------------------------------|------|
| First coat                                     |      |
| N-(1-naphthyl)-p-benzoquinoneimine             | 0.3  |
| polyvinyl chloride-acetate                     | 0.5  |
| methylethyl ketone                             | 25   |
| toluene                                        | 24.5 |
| Coated at .05 mm. on polyester film and dried. |      |
| Second coat                                    |      |
| stannous chloride                              | 1    |
| vinyl acrylate latex ("Ucar 360") (55% NVM)    | 50   |

Coated over the fully dried first coat at same wet thickness and promptly dried.

A clear image on a red background is obtained by thermographic copying procedures, but the sheet deteriorates rapidly on aging, particularly under humid storage conditions.

The thermographic copying procedure is conveniently carried out on commercially available thermographic copying machines such as the "Secretary" brand machines sold by Minnesota Mining and Manufacturing Co. and in which a copying temperature within the range of 100°-160°C. is usually attained.

Simple contact heating with heated type or stylus is also effective and permits more accurate determination of temperature if desired for comparison or test purposes.

5 What is claimed is as follows:

1. Colored sheet material capable of undergoing localized loss of color when thermographically heated in presence of a reducing agent and containing a p-quinoneimine color body in a film-forming binder, 10 wherein said color body has the structure



wherein Ar is an aromatic radical and the R, R', R'' and R''' substituent radicals may be hydrogen, halogen, alkyl, alkoxy or amido, or wherein adjacent substituent radicals may constitute a fused polycyclic or heterocyclic ring.

2. Sheet material of claim 1 disposed in face-to-face relationship with a second sheet containing said reducing agent.

3. Sheet material of claim 1 wherein is included a said reducing agent.

4. Sheet material of claim 3 wherein said reducing agent is a hydroquinone, catechol, resorcinol or trihydroxy-aromatic mild reducing agent.

5. Sheet material of claim 3 wherein said reducing agent is contained in said binder.

6. Sheet material of claim 3 wherein said reducing agent is contained in a different film-forming binder as 35 a separate stratum adjacent the stratum containing said color body.

7. Sheet material of claim 6 wherein said strata are supported on a thin flexible transparent film carrier.

\* \* \* \* \*